# EUROPEAN PATENT SPECIFICATION

(11) **EP 1 439 926 B1**
(45) Date of publication and mention of the grant of the patent: **18.05.2011**
(21) Application number: 02766948.0
(22) Date of filing: 13.09.2002
(51) Int. Cl.: B22D 11/06

(54) **CASTING STEEL STRIP METHOD AND STRIP AS SUCH**
VERFAHREN ZUM DIREKTEN BANDGIESSEN UND DIREKT GEGOSSENES STAHLBAND PER SE
Méthode de coulée directe de bande d'acier et bande coulée en tant que telle

(30) Priority: 14.09.2001 US 322261 P
(43) Date of publication of application: 28.07.2004
(73) Proprietor: NUCOR CORPORATION, Charlotte, NC 28211 (US)
(72) Inventor: BLEJDE, Walter, Brownsburg, IN 46112 (US); MAHAPATRA, Rama Ballav, New South Wales 2216 (AU); STREZOV, Lazar, Adamstown Heights, New South Wales 2289 (AU)
(74) Representative: Lerwill, John
(86) International application number: PCT/AU2002/001257
(87) International publication number: WO 2003/024644

(56) References cited:
- EP-A- 0 732 163
- WO-A-02/26422
- WO-A-98/55251
- US-A- 5 934 359
- US-A- 6 059 014
- US-A- 6 073 679
- PATENT ABSTRACTS OF JAPAN vol. 016, no. 129 (M-1228), 2 April 1992 (1992-04-02) -& JP 03 291139 A (NIPPON STEEL CORP), 20 December 1991 (1991-12-20)
- PATENT ABSTRACTS OF JAPAN vol. 014, no. 497 (C-0774), 30 October 1990 (1990-10-30) -& JP 02 205618 A (NIPPON STEEL CORP), 15 August 1990 (1990-08-15)
- PATENT ABSTRACTS OF JAPAN & JP 02 205 618 A (NIPPON STEEL CORP.) 15 August 1990
- PATENT ABSTRACTS OF JAPAN & JP 03 291 139 A (NIPPON STEEL CORP.) 20 December 1991

## Description

### TECHNICAL FIELD

This invention relates to the casting of steel strip. It has particular application to continuous casting of thin steel strip in a twin roll caster.

In twin roll casting, molten metal is introduced between a pair of contra-rotated horizontal casting rolls which are cooled so that metal shells solidify on the moving roll surfaces and are brought together at the nip between them to produce a solidified strip product delivered downwardly from the nip between the rolls. The term "nip" is used herein to refer to the general region at which the rolls are closest together. The molten metal may be poured from a ladle into a smaller vessel from which it flows through a metal delivery nozzle located above the nip so as to direct it into the nip between the rolls so forming a casting pool of molten metal supported on the casting surfaces of the rolls immediately above the nip and extending along the length of the nip. This casting pool is usually confined between side plates or dams held in sliding engagement with end surfaces of the rolls so as to dam the two ends of the casting pool against outflow, although alternative means such as electromagnetic barriers have also been proposed.

When casting thin steel strip in a twin roll caster the molten steel in the casting pool will generally be at a temperature of the order of 1500°C and above, and it is therefore necessary to achieve very high cooling rates over the casting surfaces of the rolls. It is particularly important to achieve a high heat flux and extensive nucleation on initial solidification of the steel on the casting surfaces to form the metal shells. United States Patent 5,720,336 describes how the heat flux on initial solidification can be increased by adjusting the steel melt chemistry such that a substantial proportion of the metal oxides formed as deoxidation products are liquid at the initial solidification temperature so as to form a substantially liquid layer at the interface between the molten metal and each casting surface. As disclosed in United States Patents 5,934,359 and 6,059,014 and International Application AU 99/00641, nucleation of the steel on initial solidification can be influenced by the texture of the casting surface. In particular International Application AU 99/00641 discloses that a random texture of peaks and troughs can enhance initial solidification by providing potential nucleation sites distributed throughout the casting surfaces. We have now determined that nucleation is also dependent on the presence of oxide inclusions in the steel melt and that surprisingly it is not advantageous in twin roll strip casting to cast with "clean" steel in which the number of inclusions formed during deoxidation has been minimised in the molten steel prior to casting .

Steel for continuous casting is subjected to deoxidation treatment in the ladle prior to pouring. In twin roll casting the steel is generally subjected to silicon manganese ladle deoxidation although it is possible to use aluminum deoxidation with calcium addition to control the formation of solid Al₂O₃ inclusions that can clog the fine metal flow passages in the metal delivery system through which molten metal is delivered to the casting pool. It has hitherto been thought desirable to aim for optimum steel cleanliness by ladle treatment to minimise the total oxygen level in the molten steel. However we have now determined that lowering the steel oxygen level reduces the volume of inclusions and if the total oxygen content of the steel is reduced below a certain level the nature of the initial contact between the steel and roll surfaces can be adversely effected to the extent that there is insufficient nucleation to generate rapid initial solidification and high heat flux. Molten steel is trimmed by deoxidation in the ladle such that the total oxygen content falls within a range which ensures satisfactory solidification on the casting rolls and production of a satisfactory strip product. The molten steel contains a distribution of oxide inclusions (typically MnO, CaO, SiO₂ and/or Al₂O₃) sufficient to provide an adequate density of nucleation sites on the roll surfaces for initial solidification and the resulting strip product exhibits a characteristic distribution of solidified inclusions.

### DISCLOSURE OF THE INVENTION

There is provided a method of making a steel strip by continuous casting comprising the steps of:
a. assembling a pair of cooled casting rolls having a nip between them and with confining closures adjacent the ends of the nip;
b. introducing molten low carbon steel having a total oxygen content of at least 100 ppm and a free oxygen content between 30 and 50ppm between the pair of casting rolls to form a casting pool between the casting rolls;
c. counter rotating the casting rolls and solidifying the molten steel to form metal shells on the surface of the casting rolls with levels of oxide inclusions reflected by the total oxygen content of the molten steel to promote the formation of thin steel strip; and
d. forming solidified thin steel strip through the nip of the casting rolls from said solidified shells.

The total oxygen content of the molten steel in the casting pool may be between 100 ppm and 250 ppm. More specifically, it may be about 200 ppm. The low carbon steel may have a carbon content in the range 0.001% to 0.1% by weight, a manganese content in the range 0.1% to 2.0% by weight and a silicon content in the range 0.01% to 10% by weight. The steel may have an aluminum content of the order of 0.01% or less by weight. The aluminum may for example be as little as 0.008% or less by weight. The molten steel may be a silicon/manganese killed steel.

The oxide inclusions are solidification inclusions and deoxidation inclusions. The solidification inclusions are formed during cooling and solidification of the steel in casting, and deoxidation inclusion are formed during deoxidation of the molten steel before casting. The solidified steel may contain oxide inclusions usually comprised of any one or more of MnO, SiO₂ and Al₂O₃ distributed through the steel at an inclusion density in the range 2 gm/cm³ and 4gm/cm³.

The molten steel may be refined in a ladle prior to introduction between the casting rolls to form the casting pool by heating a steel charge and slag forming material in the ladle whereby to form molten steel covered by a slag containing silicon, manganese and calcium oxides. The molten steel may be stirred by injecting an inert gas into it to cause desulphurisation, and with steels such as a silicon/manganese killed steel, then injecting oxygen, to produce steel having the desired total oxygen content of at least 100 ppm and usually less than 250 ppm. The desulphurisation may reduce the sulphur content of the molten steel to less than 0.01% by weight.

The thin steel strip produced by continuous twin roll casting as described above has a thickness of less than 5 mm and is formed of a solidified steel containing solidified oxide inclusions. The distribution of the inclusions may be such that at the two the surface regions of the strip to a depth of 2 microns from the outer faces contain solidified inclusions to a per unit area density of at least 120 inclusions/mm².

The solidified steel may be a silicon/manganese killed steel and the oxide inclusions may comprise any one or more of MnO, SiO₂ and Al₂O₃ inclusions. The inclusions typically may range in size between 2 and 12 microns, so that at least a majority of the inclusions are in that size range.

The method described above produces a unique steel high in oxygen content distributed in oxide inclusions. Specifically, the combination of the high oxygen content in the molten steel and the short residence time of the molten steel in the casting pool results in a thin steel strip with an improved ductility properties.

### BRIEF DESCRIPTION OF THE DRAWINGS

In order that the invention may be described in more detail, some specific examples will be given with reference to the accompanying drawings in which:
Figure 1 shows the effect of inclusion melting points on heat fluxes obtained in twin roll casting trials using silicon/manganese killed steels;
Figure 2 is an energy dispersive spectroscopy (EDS) map of Mn showing a band of fine solidification inclusions in a solidified steel strip;
Figure 3 is a plot showing the effect of varying manganese to silicon contents on the liquidus temperature of inclusions;
Figure 4 shows the relationship between alumina content (measured from the strip inclusions) and deoxidation effectiveness;
Figure 5 is a ternary phase diagram for MnO. SiO₂ . Al₂O₃;
Figure 6 shows the relationship between alumina content inclusions and liquidus temperature;
Figure 7 shows the effect of oxygen in a molten steel on surface tension; and
Figure 8 is a plot of the results of calculations concerning the inclusions available for nucleation at differing steel cleanliness levels.

### DETAILED DESCRIPTION OF THE PREFERRED EMBODIMENT

We have conducted extensive casting trials on a twin roll caster of the kind fully described in United States Patents 5,184,668 and 5,277,243 to produce steel strip of the order of 1 mm thick and less. Such casting trials using silicon manganese killed steel have demonstrated that the melting point of oxide inclusions in the molten steel have an effect on the heat fluxes obtained during steel solidification as illustrated in Figure 1. Low melting point oxides improve the heat transfer contact between the molten metal and the casting roll surfaces in the upper regions of the pool, generating higher heat transfer rates. Liquid inclusions are not produced when the melting point is greater than the steel temperature in the casting pool. Therefore, there is a dramatic reduction in heat transfer rate when the inclusion melting point is greater than approximately 1600°C.

Casting trials with aluminum killed steels have shown that in order to avoid the formation of high melting point alumina inclusions (melting point 2050°C) it is necessary to have calcium treatment to provide liquid CaO.Al₂O₃ inclusions.

The oxide inclusions formed in the solidified metal shells and in turn the thin steel strip comprise inclusions formed during cooling and solidification of the steel, and deoxidation inclusions formed during refining in the ladle.

The free oxygen level in the steel is reduced dramatically during cooling at the meniscus, resulting in the generation of solidification inclusions near the surface of the strip. These solidification inclusions are formed predominantly of MnO.SiO₂ by the following reaction:

Mn+Si+3O = MnO.SiO₂

The appearance of the solidification inclusions on the strip surface, obtained from an Energy Dispersive Spectroscopy (EDS) map, is shown in Figure 2. It can be seen that solidification inclusions are extremely fine (typically less than 2 to 3µm) and are located in a band located within 10 to 20µm from the surface. A typical size distribution of the inclusions through the strip is shown in Figure 3 of our paper entitled Recent Developments in Project M the Joint Development of Low Carbon Steel Strip Casting by SHP and IHI, presented at the METEC Congress 99, Dusseldorf Germany (June 13-15, 1999)

The comparative levels of the solidification inclusions is primarily determined by the Mn and Si levels in the steel. Figure 3 shows that the ratio of Mn to Si has a significant effect on the liquidus temperature of the inclusions. A manganese silicon killed steel having a carbon content in the range of 0.001% to 0.1% by weight, a manganese content in the range 0.1% to 2.0% by weight and a silicon content in the range 0.1% to 10% by weight and an aluminum content of the order of 0.01% or less by weight can produce such oxide inclusions during cooling of the steel in the upper regions of the casting pool. In particular the steel may have the following composition, termed M06:

| | |
|---|---|
| Carbon | 0.06% by weight |
| Manganese | 0.6% by weight |
| Silicon | 0.28% by weight |
| Aluminium | 0.002% by weight. |

Deoxidation inclusions are generated during deoxidation of the molten steel in the ladle with Al, Si and Mn. Thus, the composition of the oxide inclusions formed during deoxidation is mainly MnO.SiO₂ .Al₂O₃ based. These deoxidation inclusions are randomly located in the strip and are coarser than the solidification inclusions near the strip surface.

The alumina content of the inclusions has a strong effect on the free oxygen level in the steel. Figure 4 shows that with increasing alumina content, free oxygen in the steel is reduced. With the introduction of alumina, MnO. SiO₂ inclusions are diluted with a subsequent reduction in their activity, which in turn reduces the free oxygen level, as seen from the reaction below:

Mn + Si + 30 + Al₂O₃ ⇔ (Al₂O₃) .MnO.SiO₂.

For MnO-SiO₂-Al₂O₃ based inclusions, the effect of inclusion composition on liquidus temperature can be obtained from the ternary phase diagram shown in Figure 5.
Analysis of the oxide inclusions in the thin steel strip has shown that the MnO/SiO₂ ratio is typically within 0.6 to 0.8 and for this regime, it was found that alumina content of the oxide inclusions had the strongest effect on the inclusion melting point (liquidus temperature), as shown in Figure 6.

We have determined that it is important for casting in accordance with the present invention to have the solidification and deoxidation inclusions such that they are liquid at the initial solidification temperature of the steel and that the molten steel in the casting pool have an oxygen content of at least 100 ppm to produce metal shells with levels of oxide inclusions reflected by the total oxygen content of the molten steel to promote nucleation and high heat flux during the initial solidification of the steel on the casting roll surfaces. Both solidification and deoxidation inclusions are oxide inclusions and provide nucleation sites and contribute significantly to nucleation during the metal solidification process, but the deoxidation inclusions are ultimately rate controlling in that their concentration can be varied. The deoxidation inclusions are much bigger, typically greater than 4 microns, whereas the solidification inclusions are generally less than 2 microns and are MnO·SiO₂ based and have no Al₂O₃ whereas the deoxidation inclusions also have Al₂O₃.

It has been found in casting trials using the above M06 grade of silicon/manganese killed steel that if the total oxygen content of the steel is reduced in the ladle refining process to low levels of less than 100 ppm, heat fluxes are reduced and casting is impaired whereas good casting results can be achieved if the total oxygen content is at least above 100 ppm and typically on the order of 200 ppm. These oxygen levels in the ladle result in total oxygen levels of at least 70ppm and free oxygen levels between 20 and 60 ppm in the tundish, and in turn the same or slightly lower oxygen levels in the casting pool. The total oxygen content may be measured by a "Leco" instrument and is controlled by the degree of "rinsing" during ladle treatment, i.e. the amount of argon bubbled through the ladle via a porous plug or top lance, and the duration of the treatment. The total oxygen content was measured by conventional procedures using the LECO TC-436 Nitrogen/Oxygen Determinator described in the TC 436 Nitrogen/Oxygen Determinator Instructional Manual available from LECO (Form No. 200-403, Rev. Apr. 96, Section 7 at pp. 7-1 to 7-4.

In order to determine whether the enhanced heat fluxes obtained with higher total oxygen contents was due to the availability of oxide inclusions as nucleation sites, casting trials were carried out with steels in which deoxidation in the ladle was carried out with calcium silicide (Ca-Si) and the results compared with casting with the low carbon Si-killed steel known as M06 grades of steel. The results are set out in the following table:

**Table 1**

| Heat flux differences between M06 and Cal-Sil grades. | | | | |
|---|---|---|---|---|
| Cast No. | Grade | Casting speed, (m/min) | Pool Height, (mm) | Total heat Removed (MW) |
| M 33 | M06 | 64 | 171 | 3.55 |
| M 34 | M06 | 62 | 169 | 3.58 |
| O 50 | Cal-Sil | 60 | 176 | 2.54 |
| O 51 | Cal-Sil | 66 | 175 | 2.56 |

Although Mn and Si levels were similar to normal Si-killed grades, the free oxygen level in Ca-Si heats was lower and the oxide inclusions contained more CaO. Heat fluxes in Ca-Si heats were lower despite a lower inclusion melting point (See Table 2).

**Table 2**

| Slag compositions with Ca-Si deoxidation | | | | | | |
|---|---|---|---|---|---|---|
| Grade | Free Oxygen (ppm) | Slag Composition (wt %) | | | | Inclusion melting temperature (°C) |
| | | SiO₂ | MnO | Al₂O₃ | CaO | |
| Ca-Si | 23 | 32.5 | 9.8 | 32.1 | 22.1 | 1399 |

The free oxygen levels in Ca-Si grades were lower, typically 20 to 30 ppm compared to 40 to 50 ppm with M06 grades. Oxygen is a surface active element and thus reduction in oxygen level is expected to reduce the wetting between molten steel and the casting rolls and cause a reduction in the heat transfer rate. However, from Figure 7 it appears that oxygen reduction from 40 to 20 ppm may not be sufficient to increase the surface tension to levels that explain the observed reduction in the heat flux.

It can be concluded that lowering the free and total oxygen levels in the steel reduces the volume of inclusions and thus reduces the number of oxide inclusions for initial nucleation. This has the potential to adversely impact the nature of the initial contact between steel and the roll surface. Dip testing work has shown that a nucleation per unit area density of about 120/mm² is required to generate sufficient heat flux on initial solidification in the upper or meniscus region of the casting pool. Dip testing involves advancing a chilled block into a bath of molten steel at such a speed as to closely simulate the conditions at the casting surfaces of a twin roll caster. Steel solidifies onto the chilled block as it moves through the molten bath to produce a layer of solidified steel on the surface of the block. The thickness of this layer can be measured at points throughout its area to map variations in the solidification rate and therefore the effective rate of heat transfer at the various locations. It is thus possible to produce an overall solidification rate as well as total heat flux measurements. It is also possible to examine the microstructure of the strip surface to correlate changes in the solidification microstructure with the changes in observed solidification rates and heat transfer values and to examine the structures associated with nucleation on initial solidification at the chilled surface. A dip testing apparatus is more fully described in United States Patent 5,720,336.

The relationship of the oxygen content of the liquid steel on initial nucleation and heat transfer has been examined using a model described in Appendix 1. This model assumes that all the oxide inclusions are spherical and are uniformly distributed throughout the steel. A surface layer was assumed to be 2 µm and that only inclusions present in that surface layer could participate in the nucleation process on initial solidification of the steel. The input to the model was total oxygen content in the steel, inclusion diameter, strip thickness, casting speed, and surface layer thickness. The output was the percentage of inclusions of the total in the steel required to meet a targeted nucleation per unit area density of 120/mm².

Figure 8 is a plot of the percentage of oxide inclusions in the surface layer required to participate in the nucleation process to achieve the target nucleation per unit area density at different steel cleanliness levels as expressed by total oxygen content, assuming a strip thickness of 1.6 mm and a casting speed of 80/min. This shows that for a 2 µm inclusion size and 200 ppm total oxygen content, 20% of the total available oxide inclusions in the surface layer are required to achieve the target nucleation per unit area density of 120/mm². However, at 80 ppm total oxygen content, around 50% of the inclusions are required to achieve the critical nucleation rate and at 40 ppm total oxygen level there will be an insufficient level of oxide inclusions to meet the target nucleation per unit area density. Accordingly when trimming the steel by deoxidation in the ladle, the oxygen content of the steel can be controlled to produce a total oxygen content in the range 100 to 250 ppm and typically about 200 ppm. This will have the result that the two micron deep layers adjacent the casting rolls on initial solidification will contain oxide inclusions having a per unit area density of at least 120/mm². These inclusions will be present in the outer surface layers of the final solidified strip product and can be detected by appropriate examination, for example by energy dispersive spectroscopy (EDS).

### EXAMPLE

| INPUTS | | |
|---|---|---|
| Critical nucleation per unit¨area density no/mm2 (needed to achieve sufficient heat transfer rates) testing work | 120 | This value has been obtained from experimental dip |
| Roll width m | 1 | |
| Strip thickness mm | 1.6 | |
| Ladle tonnes t | 120 | |
| Steel density, kg/m3 | 7800 | |
| Total oxygen, ppm | 75 | |
| Inclusion density, kg/m3 | 3000 | |

| OUTPUTS | | |
|---|---|---|
| Mass of inclusions, kg | 21.42857 | |
| Inclusion diameter, m | 2. 00E-06 | |
| Inclusion volume, m3 | 0.0 | |
| Total no of inclusions | 1706096451319381.5 | |
| Thickness of surface layer, um (one side) | 2 | |
| Total no of inclusions surface only nucleation process | 4265241128298.4536 | These inclusions can participate in the initial |
| Casting speed, m/min | 80 | |
| Strip length, m | 9615.38462 | |
| Strip surface area, m2 | 19230.76923 | |
| Total no of nucleating sites required | 2307692.30760 | |
| % of available inclusions that need to participate in the nucleation process | 54.10462 | |

### APPENDIX 1

### List of symbols

w = roll width, m
t = strip thickness, mm
mₛ = steel weight in the ladle, tonne
ρₛ = density of steel, kg/m³
ρᵢ = density of inclusions, kg/m3
Oₜ = total oxygen in steel, ppm
d = inclusion diameter, m
vᵢ = volume of one inclusions, m3
mᵢ = mass of inclusions, kg
Nₜ = total number of inclusions
tₛ= thickness of the surface layer, um
Nₛ= total number of inclusions present in the surface (that can participate in the nucleation process)
u = casting speed, m/min
Lₛ = strip length, m
Aₛ = strip surface area, m2
N_{req}= Total number of inclusions required to meet the target nucleation density
NCₜ = target nucleation per unit area density, number/mm² (obtained
   from dip testing)
Nₐᵥ= % of total inclusions available in the molten steel at the surface of the casting rolls for initial nucleation process.

### Equations

${m}_{i} = \left({O}_{t}⁢{ x m}_{s} x 0.001\right) / 0.42$ Note: for Mn-Si killed steel, 0.42kg of oxygen is needed to produce 1 kg of neclusions with a composition of 30% MnO, 40% SiO₂ and 30% Al₂O₃.

For Al-killed steel (with Ca injection), 0.38 kg of oxygen is required to produce 1 kg of inclusions with a composition of 50% Al₂O₃ and 50% CaO. ${v}_{i} = 4.19 x {\left(d/2\right)}^{3}$ ${N}_{t} = {m}_{i} / \left({ρ}_{i}⁢{ x v}_{i}\right)$ ${N}_{s} = \left(2.0⁢{ t}_{s} x 0.001⁢{ x N}_{t}/t\right)$ ${L}_{s} = \left({m}_{s} x 1000\right) / \left({ρ}_{s} x w x t/1000\right)$ $\begin{matrix} {A}_{s} = 2.0 ⁢ { x L}_{s} x w \\ {N}_{req} = {A}_{s} x {10}^{16} ⁢ { x NC}_{t}\end{matrix}$ ${N}_{av} % = \left({N}_{req}/{N}_{s}\right) x 100.0$
Eq. 1 calculates the mass of inclusions in steel.
Eq. 2 calculates the volume of one inclusion assuming they are spherical.
Eq. 3 calculates the total number of inclusions available in steel.
Eq. 4 calculates the total number of inclusions available in the surface layer (assumed to be 2 um on each side). Note that these inclusions can only participate in the initial nucleation.
Eq. 5 and Eq. 6 used to calculate the total surface area of the strip.
Eq. 7 calculates the number of inclusions needed at the surface to meet the target nucleation rate.
Eq. 8 is used to calculate the percentage of total inclusions available at the surface which must participate in the nucleation process. Note if this number is great than 100%, then the number of inclusions at the surface is not sufficient to meet target nucleation rate.

## Claims

1. A method of making a steel strip by continuous casting comprising the steps of:
a. assembling a pair of cooled casting rolls having a nip between them and with confining closures adjacent the ends of the nip;
b. introducing molten low carbon steel having a total oxygen content of at least 100 ppm and a free oxygen content between 30 and 50ppm between the pair of casting rolls to form a casting pool between the casting rolls;
c. counter rotating the casting rolls and solidifying the molten steel to form metal shells on the surface of the casting rolls with levels of oxide inclusions reflected by the total oxygen content of the molten steel to promote the formation of thin steel strip; and
d. forming solidified thin steel strip through the nip of the casting rolls from said solidified shells.

2. A method of making steel strip as claimed in Claim 1, wherein the molten steel in the casting pool has carbon content in the range of 0.001% to 0.01% by weight, a manganese content in the range of 0.01% to 2.0% by weight, and a silicon content in the range of 0.01% to 10% by weight.

3. A method of making steel strip as claimed in Claim 2 wherein the molten steel in the casting pool has an aluminum content on the order of 0.01% or less by weight.

4. A method of making steel strip as claimed any one of the preceding claims, wherein the molten steel in the casting pool has an oxygen content between 100 ppm and 250 ppm.

5. A method of making steel strip as claimed in any one of the preceding claims, wherein the molten steel contains oxide inclusions comprising any one or more of MnO, SiO₂ and Al₂O₃ distributed through the steel at an inclusion density in the range 2 gm/cm³ to 4 gm/cm³.

6. A method of making steel strip as claimed in any one of the preceding claims, wherein more than a majority of the inclusions range in size between 2 and 12 microns.

7. A method of making steel strip as claimed in any one of the preceding claims, wherein the sulphur content of the molten steel is less than 0.01% by weight.

8. A method of making steel strip as claimed in Claim 1, comprising the additional steps of:
e. refining the molten steel in the ladle prior to forming the casting pool by heating a steel charge and slag forming material in the ladle to form molten steel covered by a slag containing silicon, manganese and calcium oxides, stirring the molten steel in the ladle by injecting an inert gas into molten steel to cause desulphurisation, and thereafter injecting oxygen to produce molten steel having the total oxygen content of greater than 100ppm.

9. A method of making steel strip as claimed in Claim 8, wherein the desulphurisation reduces the sulphur content of the molten steel to less than 0.01% by weight.

10. A method of making a thin steel strip as claimed in Claim 8 or 9, wherein the solidified steel is a silicon/manganese killed steel and the inclusions comprise any one or more of MnO, SiO₂ and Al₂O₃.

11. A method of making a thin steel strip as claimed in any one of Claims 8 to 10, wherein more than a majority of the inclusions range in size between 2 and 12 microns.

12. A method of making a steel strip as claimed in any one of Claims 8 to 11, wherein the solidified steel has a total oxygen content in the range of 100 ppm to 250 ppm.

13. A thin steel strip produced by twin roll casting to a thickness of less than 5mm and formed of a solidified steel containing solidified oxide inclusions distributed such that at surface regions of the strip to a depth of 2 microns from the surface contain such inclusions to a per unit area density of at least 120 inclusions/mm².

14. A thin steel strip as claimed in Claim 13, wherein the majority of the solidified steel is a silicon/manganese killed steel and the inclusions comprise any one or more of MnO, SiO₂ and Al₂O₃.

15. A thin steel strip as claimed in Claim 13 or Claim 14, wherein the majority of the inclusions range in size between 2 and 12 microns.

16. A thin steel strip as claimed in any one of Claims 13 to 15, wherein the solidified steel has an oxygen content reflective of total oxygen content in the range 100 ppm to 250 ppm and a free oxygen content between 30 and 50ppm in the molten steel from which the strip is made.

17. A thin steel strip produced by twin roll casting to a thickness of less than 5 mm and formed of a solidified steel containing oxide inclusions distributed to reflect a total oxygen content in the range 100 ppm to 250 ppm and a free oxygen content between 30 and 50ppm in the molten steel from which the strip is made.

18. A thin steel strip as claimed in Claim 17, wherein the majority of the solidified steel is a silicon/manganese killed steel and the inclusions comprise any one or more of MnO, SiO₂ and Al₂O₃.

19. A thin steel strip as claimed in Claim 17 or Claim 18, wherein the majority of the inclusions range in size between 2 and 12 microns.

## Patentansprüche

1. Verfahren zur Herstellung eines Stahlbands durch Stranggießen, umfassend die folgenden Schritte:
a. Montieren eines Paars von gekühlten Gießwalzen mit einem Walzenspalt dazwischen und mit beschränkenden Verschlüssen neben den Enden des Walzenspalts;
b. Einbringen von geschmolzenem Stahl mit niedrigem Kohlenstoffgehalt, der einen gesamten Sauerstoffgehalt von mindestens 100 ppm und einen freien Sauerstoffgehalt zwischen 30 und 50 ppm aufweist, zwischen das Paar von Gießwalzen, um zwischen den Gießwalzen ein Gießbad zu bilden;
c. gegenläufiges Drehen der Gießwalzen und Verfestigen des geschmolzenen Stahls, um an der Oberfläche der Gießwalzen Metallschalen mit Sauerstoffeinschlussraten, die durch den gesamten Sauerstoffgehalt des geschmolzenen Stahls widergespiegelt werden, zu bilden, um die Bildung eines dünnen Stahlbands zu fördern; und
d. Bilden eines verfestigten dünnen Stahlbands durch den Walzenspalt der Gießwalzen aus den verfestigten Schalen.

2. Verfahren zur Herstellung eines Stahlbands nach Anspruch 1, wobei der geschmolzene Stahl im Gießbad einen Kohlenstoffgehalt im Bereich von 0,001 bis 0,01 Gew.%, einen Mangangehalt im Bereich von 0,01 bis 2,0 Gew.%, und einen Siliziumgehalt im Bereich von 0,01 bis 10 Gew.% aufweist.

3. Verfahren zur Herstellung eines Stahlbands nach Anspruch 2, wobei der geschmolzene Stahl im Gießbad einen Aluminiumgehalt in der Größenordnung von 0,01 Gew.% oder weniger aufweist.

4. Verfahren zur Herstellung eines Stahlbands nach einem der vorhergehenden Ansprüche, wobei der geschmolzene Stahl im Gießbad einen Sauerstoffgehalt zwischen 100 ppm und 250 ppm aufweist.

5. Verfahren zur Herstellung eines Stahlbands nach einem der vorhergehenden Ansprüche, wobei der geschmolzene Stahl Sauerstoffeinschlüsse enthält, die eines oder mehrere aus MnO, SiO₂ und Al₂O₃ umfassen und mit einer Einschlussdichte im Bereich von 2 g/cm³ bis 4 g/cm³ über den Stahl hinweg verteilt sind.

6. Verfahren zur Herstellung eines Stahlbands nach einem der vorhergehenden Ansprüche, wobei ein Großteil der Einschlüsse in einem Größenbereich zwischen 2 und 12 Mikron liegt.

7. Verfahren zur Herstellung eines Stahlbands nach einem der vorhergehenden Ansprüche, wobei der Schwefelgehalt des geschmolzenen Stahls geringer als 0,01 Gew.% ist.

8. Verfahren zur Herstellung eines Stahlbands nach Anspruch 1, umfassend die folgenden zusätzlichen Schritte:
e. Veredeln des geschmolzenen Stahls in der Pfanne, bevor das Gießbad gebildet wird, indem eine Stahlladung und ein Schlacke bildendes Material in der Pfanne erhitzt werden, um geschmolzenen Stahl zu bilden, der von einer Schlacke bedeckt ist, die Silizium-, Mangan- und Calciumoxid enthält, Rühren des geschmolzenen Stahls in der Pfanne durch Einspritzen eines Inertgases in den geschmolzenen Stahl, um eine Entschwefelung zu bewirken, und danach Einspritzen von Sauerstoff, um geschmolzenen Stahl zu erzeugen, der den gesamten Sauerstoffgehalt von mehr als 100 ppm aufweist.

9. Verfahren zur Herstellung eines Stahlbands nach Anspruch 8, wobei die Entschwefelung den Schwefelgehalt des geschmolzenen Stahls auf weniger als 0,01 Gew.% verringert.

10. Verfahren zur Herstellung eines Stahlbands nach Anspruch 8 oder 9, wobei der verfestigte Stahl ein silizium/manganberuhigter Stahl ist und die Einschlüsse eines oder mehrere aus MnO, SiO₂ und Al₂O₃ umfassen.

11. Verfahren zur Herstellung eines Stahlbands nach einem der Ansprüche 8 bis 10, wobei ein Großteil der Einschlüsse in einem Größenbereich zwischen 2 und 12 Mikron liegt.

12. Verfahren zur Herstellung eines Stahlbands nach einem der Ansprüche 8 bis 11, wobei der verfestigte Stahl einen gesamten Sauerstoffgehalt im Bereich von 100 ppm bis 250 ppm aufweist.

13. Dünnes Stahlband, das durch einen Doppelwalzenguß mit einer Dicke von weniger als 5 mm hergestellt ist und aus einem verfestigten Stahl gebildet ist, der verfestigte Oxideinschlüsse enthält, die so verteilt sind, dass diese Einschlüsse in Oberflächenbereichen des Bands bis zu einer Tiefe von 2 Mikron von der Oberfläche in einer Dichte pro Einheitsfläche von mindestens 120 Einschlüssen/mm² enthalten sind.

14. Dünnes Stahlband nach Anspruch 13, wobei der Großteil des verfestigten Stahls ein silizium/manganberuhigter Stahl ist und die Einschlüsse eines oder mehrere aus MnO, SiO₂ und Al₂O₃ umfassen.

15. Dünnes Stahlband nach Anspruch 13 oder Anspruch 14, wobei der Großteil der Einschlüsse in einem Größenbereich zwischen 2 und 12 Mikron liegt.

16. Dünnes Stahlband nach einem der Ansprüche 13 bis 15, wobei der verfestigte Stahl einen Sauerstoffgehalt aufweist, der den gesamten Sauerstoffgehalt in der Größenordnung von 100 ppm bis 250 ppm und einen freien Sauerstoffgehalt zwischen 30 und 50 ppm im geschmolzenen Stahl, aus dem das Band hergestellt ist, widerspiegelt.

17. Dünnes Stahlband, das durch einen Doppelwalzenguß mit einer Dicke von weniger als 5 mm hergestellt ist und aus einem verfestigten Stahl gebildet ist, der Sauerstoffeinschlüsse enthält, die so verteilt sind, dass sie einen gesamten Sauerstoffgehalt im Bereich von 100 ppm bis 250 ppm und einen freien Sauerstoffgehalt zwischen 30 und 50 ppm im geschmolzenen Stahl, aus dem das Band hergestellt ist, widerspiegeln.

18. Dünnes Stahlband nach Anspruch 17, wobei der Großteil des verfestigten Stahls ein silizium/manganberuhigter Stahl ist und die Einschlüsse eines oder mehrere aus MnO, SiO₂ und Al₂O₃ umfassen.

19. Dünnes Stahlband nach Anspruch 17 oder Anspruch 18, wobei der Großteil der Einschlüsse in einem Größenbereich zwischen 2 und 12 Mikron liegt.

## Revendications

1. Procédé de fabrication d'une bande d'acier par coulée continue comprenant les étapes consistant à :
a. assembler une paire de cylindres de coulée refroidis ayant un écartement entre cylindres entre eux et avec des fermetures de confinement adjacentes aux extrémités de l'écartement entre cylindres ;
b. introduire de l'acier bas carbone fondu ayant une teneur en oxygène totale d'au moins 100 ppm et une teneur en oxygène libre entre 30 et 50 ppm entre la paire de cylindres de coulée pour former un bassin de coulée entre les cylindres de coulée ;
c. tourner en sens opposé les cylindres de coulée et solidifier l'acier fondu pour former des coques de métal sur la surface des cylindres de coulée avec des niveaux d'inclusions d'oxyde réfléchis par la teneur en oxygène totale de l'acier fondu pour promouvoir la formation d'une bande d'acier mince ; et
d. former une bande d'acier mince solidifiée à travers l'écartement entre cylindres des cylindres de coulée à partir desdites coques solidifiées.

2. Procédé de fabrication d'une bande d'acier selon la revendication 1, dans lequel l'acier fondu dans le bassin de coulée a une teneur en carbone dans la plage entre 0.001% et 0.01% en poids, une teneur en manganèse dans la plage entre 0.01% et 2.0% en poids, et une teneur en silicium dans la plage entre 0.01% et 10% en poids.

3. Procédé de fabrication d'une bande d'acier selon la revendication 2, dans lequel l'acier fondu dans le bassin de coulée a une teneur en aluminium de l'ordre de 0.01% ou inférieur en poids.

4. Procédé de fabrication d'une bande d'acier selon une quelconque des revendications précédentes, dans lequel l'acier fondu dans le bassin de coulée a une teneur en oxygène comprise entre 100 ppm et 250 ppm.

5. Procédé de fabrication d'une bande d'acier selon une quelconque des revendications précédentes, dans lequel l'acier fondu contient des inclusions d'oxyde comprenant n'importe lequel de un ou plusieurs de MnO, SiO₂ et Al₂O₃ distribués à travers l'acier à une densité d'inclusion dans la plage entre 2 gm/cm³ et 4 gm/cm³.

6. Procédé de fabrication d'une bande d'acier selon une quelconque des revendications précédentes, dans lequel plus d'une majorité des inclusions ont une taille comprise dans une plage de 2 à 12 microns.

7. Procédé de fabrication d'une bande d'acier selon une quelconque des revendications précédentes, dans lequel la teneur en sulfure de l'acier fondu est inférieure à 0.01% en poids.

8. Procédé de fabrication d'une bande d'acier selon la revendication 1, comprenant les étapes additionnelles consistant à :
e. raffiner l'acier fondu dans la poche de coulée avant de former le bassin de coulée en chauffant une charge d'acier et le matériau formant le laitier de fonderie dans la poche de coulée pour former l'acier fondu couvert par un laitier contenant des oxydes de silicium, manganèse et calcium, agiter l'acier fondu dans la poche en injectant un gaz inerte dans l'acier fondu pour provoquer une désulfuration, et ensuite injecter de l'oxygène pour produire de l'acier fondu ayant la teneur en oxygène totale supérieure à 100 ppm.

9. Procédé de fabrication d'une bande d'acier selon la revendication 8, dans lequel la désulfuration réduit la teneur en sulfure de l'acier fondu à moins de 0.01% en poids.

10. Procédé de fabrication d'une bande d'acier mince selon la revendication 8 ou 9, dans lequel l'acier solidifié est un acier calmé au silicium/manganèse et les inclusions comprennent n'importe lequel ou plusieurs de MnO, SiO₂ et Al₂O₃.

11. Procédé de fabrication d'une bande d'acier mince selon une quelconque des revendications 9 à 10, dans lequel plus d'une majorité des inclusions ont une taille comprise dans une plage de 2 à 12 microns.

12. Procédé de fabrication d'une bande d'acier selon une quelconque des revendications 8 à 11, dans lequel l'acier solidifié a une teneur en oxygène totale comprise entre 100 ppm et 250 ppm.

13. Bande d'acier mince produite par coulée dans des cylindres jumeaux à une épaisseur de moins de 5 mm et formée d'un acier solidifié contenant des inclusions d'oxyde solidifiées distribuées de telle sorte que à des régions de surface de la bande à une profondeur de 2 microns à partir de la surface contiennent de telles inclusions à une densité par zone unitaire d'au moins 120 inclusions/mm².

14. Bande d'acier mince selon la revendication 13, dans laquelle la majorité de l'acier solidifié est un acier calmé au silicium/manganèse et les inclusions comprennent n'importe lequel ou plusieurs de MnO, SiO₂ et Al₂O₃.

15. Bande d'acier mince selon la revendication 13 ou 14, dans laquelle la majorité des inclusions ont une taille comprise dans une plage de 2 à 12 microns.

16. Bande d'acier mince selon une quelconque des revendications 13 à 15, dans laquelle l'acier solidifié a une teneur en oxygène qui réfléchit la teneur en oxygène totale dans la plage de 100 ppm à 250 ppm et une teneur en oxygène libre comprise entre 30 et 50 ppm dans l'acier fondu à partir duquel la bande est fabriquée.

17. Bande d'acier mince produit par coulée dans des cylindres jumeaux à une épaisseur de moins de 5 mm et formée d'un acier solidifié contenant des inclusions d'oxyde distribuées pour réfléchir une teneur en oxygène totale dans la plage de 100 ppm à 250 ppm et une teneur en oxygène libre comprise entre 30 et 50 ppm dans l'acier fondu à partir duquel la bande est fabriquée.

18. Bande d'acier mince selon la revendication 17, dans laquelle la majorité de l'acier solidifié est un acier calmé au silicium/manganèse et les inclusions comprennent n'importe lequel ou plusieurs de MnO, SiO₂ et Al₂O₃.

19. Bande d'acier mince selon la revendication 17 ou 18, dans laquelle la majorité des inclusions ont une taille comprise entre 2 et 12 microns.
